# EUROPEAN PATENT SPECIFICATION

(11) **EP 3 770 322 B1**
(45) Date of publication and mention of the grant of the patent: **20.05.2026**
(21) Application number: 19219097.3
(22) Date of filing: 20.12.2019
(51) Int. Cl.: D21H 21/22, D21C 5/00, D21C 9/153, D21H 11/10, D21H 17/00, D21H 21/32

(54) **METHOD FOR IMPROVING FIBER SOFTNESS OF HIGH YIELD PULP**
VERFAHREN ZUR VERBESSERUNG DER FASERWEICHHEIT VON ZELLSTOFF MIT HOHER AUSBEUTE
PROCÉDÉ POUR AMÉLIORER LA DOUCEUR DE FIBRES DE PÂTE À HAUT RENDEMENT

(30) Priority: 24.07.2019 CN 201910672286
(43) Date of publication of application: 27.01.2021
(73) Proprietor: Zhejiang Jingxing Paper Joint Stock Co., Ltd., 314214 Pinghu City, Zhejiang (CN)
(72) Inventor: Cao, Haibing, Pinghu City, Zhejiang, 314214 (CN); An, Xingye, Pinghu City, Zhejiang, 314214 (CN); Lu, Bin, Pinghu City, Zhejiang, 314214 (CN); Liu, Hongbin, Pinghu City, Zhejiang, 314214 (CN); Zhang, Runqing, Pinghu City, Zhejiang, 314214 (CN); Xu, Dong, Pinghu City, Zhejiang, 314214 (CN); Dong, Hongming, Pinghu City, Zhejiang, 314214 (CN)
(74) Representative: 2s-ip Schramm Schneider Bertagnoll Patent- und Rechtsanwälte Part mbB

(56) References cited:
- WO-A1-2013/188657
- WO-A1-2014/029909
- WO-A1-2016/080895
- WO-A1-95/13415
- WO-A1-96/00811
- CN-A- 108 071 038
- US-A1- 2006 102 299

## Description

### FIELD

The present disclosure relates to improving fiber softness of high yield pulp.

### BACKGROUND

As a pulping technology with high yield, high quality, and low pollution, the chemimechanical pulping process emerged in 1970s, which is one kind of high yield pulping. The high yield pulp obtained from high yield pulping has characteristics of high yield and low pollution, such that a paper factory can manufacture products with premium quality at a lower cost. It can be said that high yield pulp fills up the blank between conventional mechanical pulp and chemical pulp in respect of performance. In recent years, owing to its so many functional advantages in papermaking, such as high bulk factor, high stiffness, large opacity, good dimensional stability, and good printability, etc. the high yield pulp has gained wide applications in various kinds of paper and paper boards.

With improvement of quality of life, people focus more and more on paper softness, which gradually exposes the drawback of high yield pulp, i.e. poor softness, one of bottlenecks restricting development of the high yield pulp. The Chinese patent No. 2016105224934 discloses a method of manufacturing a paper towel containing high yield pulp, comprising: subjecting the high yield pulp to refiner beating through a crushing-type beating process, wherein the beating consistency is 20%, and the freeness of the pulp is controlled to 250~400ml. On the one hand, pretreating the high yield pulp using the crushing-type beating process will reduce the volume of fiber cavities, thereby affecting the water retention value of pulp fibers and water- absorptivity of paper towels; and on the other hand, the crushing pretreatment has less impact on lignin of the fiber, thereby affecting inter-fiber bonding force in the paper towel and reducing the mechanical strength of the paper towel.

WO2013 /188657 A1 relates to an energy efficient process for forming cellulose nanofibers from a cellulosic material, comprising: treating the cellulosic material with an aqueous slurry containing a depolymerizing agent selected from (a) ozone at a charge level of at least about 0.1 wt/wt%, based on the dry weight of the cellulosic material for generating free radicals in the slurry; (b) a cellulase enzyme at a concentration from about 0.1 to about 10 lbs/ton based on the dry weight of the cellulosic material; or (c) a combination of both (a) and (b), under conditions sufficient to cause partial depolymerization of the cellulosic material; and concurrently or subsequently comminuting the cellulosic material to liberate cellulose nanofibers; wherein the overall process achieves an energy efficiency (as defined herein) of at least about 2%.

US 2006/102299 A1 relates to a process of enzymatic deinking of waste papers.

WO 2014/029909 A1 relates to a method and intermediate for the production of highly refined or microfibrillated cellulose.

### SUMMARY

An object of the present invention is to improve fiber softness of high yield pulp, which enables removal of part of lignin from the high yield pulp fiber to thereby improve fiber softness.

According to the invention, this object is achieved by the subject-matter as defined in claim 1. Advantageous embodiments of the invention are defined in the dependent claims. Thus, the present invention provides the use of ozone and cellulase to improve fiber softness of a high yield pulp, which use enables removal of part of lignin from the high yield pulp, including a high yield pulp with a pulp consistency of 1~3%, comprising steps of:
Step 1: treating the high yield pulp with ozone, wherein the concentration of ozone is 10~30%, the treatment temperature is 30~50°C, the treatment duration is 60~210s, and the pH value during treatment is 2.5~4.5;
Step 2: treating the treated high yield pulp from step 1 with cellulase, wherein the content of cellulase is 0.1~3EGU/g, the treatment duration is 30~60min, the temperature during treatment is 45~60°C.

Preferably, the treatment temperature in step 1 is 30°C, 35°C, 40°C, 45°C or 50°C, respectively; the concentration of ozone is 10%; the treatment duration is 120s, the pH value during treatment is 3, and the consistency of the high yield pulp is 2%.

Preferably, the consistency of high yield pulp in step 1 is 1.5%, 2%, 2.5%, 3% or 3.5%, respectively; the treatment temperature is 30°C, the concentration of ozone is 10%; the treatment duration is 120s, the pH value during treatment is 3.

Preferably, the temperature when treating the high yield pulp with ozone is controlled and adjusted by the temperature of the water bath.

Preferably, the cellulase reacts with the high yield pulp in a 1000ml beaker.

Preferably, the cellulase in step 2 includes one of or a mixture of at least two of endoglucanase, exoglucanase, and β-glycosidase.

In view of the above, the present disclosure offers the following advantages: the high yield pulp in the present disclosure is sequentially treated with ozone and cellulase. Because the ozone has a relatively low dissolvability, it can hardly enter the inside of the fiber; therefore, it first acts on the fiber surface such that ozonation attacks the primary wall lignin, the outer wall of the secondary wall and the intercellular lignin, wherein the lignin side chain is oxidized (by polymer depolymerization), the aromatic ring is broken (ring-opened), forming an organic acid which is dissolved in water. With loss of yield, the primary wall and the intercellular layer selectively remove lignin and expose the surface hydrophilic substances. The removal of lignin on the surface increases the softness of the fiber and loosens the fiber structure.

Therefore, treating the fiber with ozone can open a "channel" for the entry of cellulase. Then the cellulase can hydrolyze the amorphous region of fiber, allowing water molecules to enter the fiber, and the distance between fiber macromolecule chains increases, which causes the fiber to deform with reduced stiffness, thereby improving the softness. Therefore, by treating with cellulase based on the pretreatment of high-yield pulp with ozone, the present disclosure increases the accessibility of cellulase and fiber. With an intention to reduce use of cellulase and improve the post-treatment fiber softness, the present disclosure offers a dual-beneficial and prospective process for treating high yield pulp; besides, ozone as a green agent can improve the softness of the fiber without or with little pollution to the environment.

### BRIEF DESCRIPTION OF THE DRAWINGS

Hereinafter, the present disclosure will be further illustrated with reference to the accompanying drawings:
Fig. 1 shows a schematic diagram of softness with ozone under different temperatures;
Fig. 2 shows a schematic diagram of softness with ozone under different pulp consistencies.

### DETAILED DESCRIPTION OF EMBODIMENTS

A method for improving fiber softness of high yield pulp, including a high yield pulp with a pulp consistency of 1~3%, the method comprising steps of:
Step 1: treating the high yield pulp with ozone, wherein the concentration of ozone is 10~30%, the treatment temperature is 30~50°C, the treatment duration is 60~210s, and the pH value during treatment is 2.5~4.5;
Step 2: treating the treated high yield pulp from step 1 with cellulase, wherein the content of cellulase is 0.1~3EGU/g, the treatment duration is 30~60min, the temperature during treatment is 45~60°C.

The high yield pulp in the present disclosure is sequentially treated with ozone and cellulase. Because the ozone has a relatively low dissolvability, it can hardly enter the inside of the fiber; therefore, it first acts on the fiber surface such that ozonation attacks the primary wall lignin, the outer wall of the secondary wall and the intercellular lignin, wherein the lignin side chain is oxidized (by polymer depolymerization), the aromatic ring is broken (ring-opened), forming an organic acid which is dissolved in water. With loss of yield, the primary wall and the intercellular layer selectively remove lignin and expose the surface hydrophilic substances. The removal of lignin on the surface increases the softness of the fiber and loosens the fiber structure. Therefore, treating the fiber with ozone can open a "channel" for the entry of cellulase. Then the cellulase can hydrolyze the amorphous region of fiber, allowing water molecules to enter the fiber, and the distance between fiber macromolecule chains increases, which causes the fiber to deform with reduced stiffness, thereby improving the softness. Therefore, by treating with cellulase based on the pretreatment of high-yield pulp with ozone, the present disclosure increases the accessibility of cellulase and fiber. With an intention to reduce use of cellulase and improve the post-treatment fiber softness, the present disclosure offers a dual-beneficial and prospective process for treating high yield pulp; besides, ozone as a green agent can improve the softness of the fiber without or with little pollution to the environment.

The temperature for treating the high-yield pulp with ozone is controlled via a water bath. The water bath is simple to operate and has a good heating effect, such that it may guarantee that the adjusted temperature reaches the set temperature range to thereby guarantee the thermostatic effect of the temperature. The ozone reacts with the high yield pulp via a three-neck flask, which is convenient for adjusting ozone concentration and pH value during the test; the adjustment of the ozone concentration can be independent from the adjustment of pH value, thereby improving the efficiency of adjustment. The cellulase reacts with the high yield pulp via a 1000ml beaker, which facilitates stirring during the cellulase treatment to thereby improve the treatment effect; the cellulase in step two includes one of or a mixture of at least two of endoglucanase, exoglucanase, and β-glycosidase, which may be adjusted according to different high-yield pulps so as to meet different needs, thereby offering a good applicability.

### First Example:

A method for improving fiber softness of high yield pulp, including a high yield pulp with a pulp consistency of 2%, the method comprising steps of:
Step 1: treating the high yield pulp with ozone, wherein the treatment temperature was 30°C, 35°C, 40°C, 45°C or 50°C, respectively; the concentration of ozone was 10%; the treatment duration was 120s, the pH value during treatment was 3, and the consistency of the high yield pulp was 2%;
Step 2: treating the treated high yield pulp from step 1 with cellulase, wherein the content of cellulase was 0.5EGU/g, the treatment duration was 30min, the pH value during treatment was 45°C.

The treated high yield pulp was subjected to softness detection, wherein the curve relationship between the detected softness and the treatment temperatures is shown in Fig. 1.

### Second Example:

A method for improving fiber softness of high yield pulp, including a high yield pulp with a pulp consistency of 2%, the method comprising steps of:
Step 1: treating the high yield pulp with ozone, wherein the treatment temperature was 30°C; the concentration of ozone was 10%; the treatment duration was 120s, the _{P}H value during treatment was 3, and the consistency of the high yield pulp was 1.5%, 2%, 2.5%, or 3%, respectively;
Step 2: treating the treated high yield pulp from step 1 with cellulase, wherein the content of cellulase was 0.5EGU/g, the treatment duration was 30min, the temperature during treatment was 45°C.

The treated high yield pulp was subjected to softness detection, wherein the curve relationship between the detected softness and the consistencies of the high yield pulp is shown in Fig. 2.

Additionally, the ozone treatment in step 1 may also treat the high yield pulp by changing the ozone consistency, or the ozone treatment duration, or the pH value during treatment.

## Claims

1. Use of ozone and cellulase to improve fiber softness of a high yield pulp, which use enables removal of part of lignin from the high yield pulp, including a high yield pulp with a pulp consistency of 1~3%, comprising steps of:
Step 1: treating the high yield pulp with ozone, wherein the concentration of ozone is 10~30%, the treatment temperature is 30~50°C, the treatment duration is 60~210s, and the pH value during treatment is 2.5~4.5;
Step 2: treating the treated high yield pulp from step 1 with cellulase, wherein the content of cellulase is 0.1 ~ 3EGU/g, the treatment duration is 30~60min and the treatment temperature is 45~60°C.

2. The use according to claim 1, wherein the treatment temperature in step 1 is 30°C, 35°C, 40°C, 45°C or 50°C, respectively; the concentration of ozone is 10%; the treatment duration is 120s, the pH value during treatment is 3, and the consistency of the high yield pulp is 2%.

3. The use according to claim 1, wherein the consistency of high yield pulp in step 1 is 1.5%, 2%, 2.5%, 3% or 3.5%, respectively; the treatment temperature is 30°C, the concentration of ozone is 10%; the treatment duration is 120s, the pH value during treatment is 3.

4. The use according to any one of claims 1~3, wherein the temperature when treating the high yield pulp with ozone is controlled and adjusted by the temperature of a water bath.

5. The use according to any one of claims 1~3, wherein the cellulase reacts with the high yield pulp in a 1000ml beaker.

6. The use according to claim 1, wherein the cellulase in step 2 includes one of or a mixture of at least two of endoglucanase, exoglucanase, and β-glycosidase.

## Patentansprüche

1. Verwendung von Ozon und Cellulase zur Verbesserung der Faserweichheit eines Hochausbeutezellstoffs, wobei diese Verwendung die Entfernung eines Teils des Lignins aus dem Hochausbeutezellstoff ermöglicht, einschließlich eines Hochausbeutezellstoffs mit einer Stoffkonsistenz von 1-3 %, umfassend die Schritte:
Schritt 1: Behandeln des Hochausbeutezellstoffs mit Ozon, wobei die Ozonkonzentration 10-30 % beträgt, die Behandlungstemperatur 30-50 °C, die Behandlungsdauer 60-210 s und der pH-Wert während der Behandlung 2,5-4,5 beträgt;
Schritt 2: Behandeln des behandelten Hochausbeutezellstoffs aus Schritt 1 mit Cellulase, wobei der Gehalt an Cellulase 0,1 bis 3 EGU/g beträgt, die Behandlungsdauer 30 bis 60 min und die Behandlungstemperatur 45 bis 60°C.

2. Verwendung nach Anspruch 1, wobei die Behandlungstemperatur in Schritt 1 jeweils 30°C, 35°C, 40°C, 45°C oder 50°C beträgt; die Ozonkonzentration 10% beträgt; die Behandlungsdauer 120s beträgt, der pH-Wert während der Behandlung 3 beträgt und die Konsistenz des Hochausbeutezellstoffs 2% beträgt.

3. Verwendung nach Anspruch 1, wobei die Konsistenz von Hochausbeutezellstoff in Schritt 1 jeweils 1,5 %, 2 %, 2,5 %, 3 % oder 3,5 % beträgt; die Behandlungstemperatur 30 ° C beträgt, die Ozonkonzentration 10 % beträgt; die Behandlungsdauer 120 s beträgt, der pH-Wert während der Behandlung 3 beträgt.

4. Verwendung nach einem der Ansprüche 1 bis 3, wobei die Temperatur bei der Behandlung des Hochausbeutezellstoffs mit Ozon durch die Temperatur eines Wasserbads gesteuert und geregelt wird.

5. Verwendung nach einem der Ansprüche 1 bis 3, wobei die Cellulase mit dem Hochausbeutezellstoff in einem 1000-ml-Becherglas reagiert.

6. Verwendung nach Anspruch 1, wobei die Cellulase eine von Endoglucanase, Exoglucanase und β-Glykosidase oder ein Gemisch aus mindestens zwei davon umfasst.

## Revendications

1. Utilisation d'ozone et de cellulase pour améliorer la douceur des fibres d'une pâte à haut rendement, ladite utilisation permettant l'élimination d'une partie de lignine de la pâte à haut rendement, comportant une pâte à haut rendement présentant une consistance de pâte de 1 à 3 %, comprenant les étapes de :
étape 1 : traitement de la pâte à haut rendement avec de l'ozone, la concentration d'ozone étant de 10 à 30 %, la température de traitement étant de 30 à 50 °C, la durée de traitement étant de 60 à 210 s et la valeur de pH durant le traitement étant de 2,5 à 4,5 ;
étape 2 : traitement de la pâte à haut rendement traitée de l'étape 1 avec de la cellulase, la teneur en cellulase étant de 0,1 à 3 EGU/g, la durée de traitement étant de 30 à 60 min et la température de traitement étant de 45 à 60 °C.

2. Utilisation selon la revendication 1, dans laquelle la température de traitement dans l'étape 1 est de 30 °C, 35 °C, 40°C, 45 °C ou 50 °C respectivement ; la concentration d'ozone est de 10 %, la durée de traitement est de 120 s, la valeur de pH durant le traitement est de 3 et la consistance de la pâte à haut rendement est de 2 %.

3. Utilisation selon la revendication 1, dans laquelle la consistance de la pâte à haut rendement dans l'étape 1 est de 1,5 %, 2 %, 2,5 %, 3 % ou 3,5 % respectivement ; la température de traitement est de 30 °C, la concentration d'ozone est de 10 % ; la durée de traitement est de 120 s, la valeur de pH durant le traitement est de 3.

4. Utilisation selon l'une quelconque des revendications 1 à 3, dans laquelle la température lors du traitement de la pâte à haut rendement avec de l'ozone est contrôlée et ajustée par la température d'un bain-marie.

5. Utilisation selon l'une quelconque des revendications 1 à 3, dans laquelle la cellulase réagit avec la pâte à haut rendement dans un bêcher de 1000 ml.

6. Utilisation selon la revendication 1, dans laquelle la cellulase dans l'étape 2 comporte une substance ou un mélange d'au moins deux substances parmi l'endoglucanase, l'exoglucanase et la β-glycosidase.
